

April 2, 1963

J. S. HILL

3,083,445

METHOD OF MAKING AN ELECTRICAL RESISTANCE DEVICE

Filed Aug. 8, 1957

Fig. 1.



Fig. 2.



INVENTOR.

JAMES S. HILL  
BY *Mark Miller*  
James S. Bryan  
ATTORNEYS

## 1

3,083,445

METHOD OF MAKING AN ELECTRICAL  
RESISTANCE DEVICE

James S. Hill, Cranford, N.J., assignor, by mesne assignments, to Engelhard Industries, Inc., Newark, N.J., a corporation of Delaware

Filed Aug. 8, 1957, Ser. No. 676,951  
5 Claims. (Cl. 29—155.62)

The present invention deals with an electrical resistance device and more particularly with an electrically heated muffle for muffle type furnaces.

Electrical furnaces of the muffle type comprise an insulated housing containing an elongated hollow muffle of suitable electrical insulating and heat conductive refractory material, such as Alundum, with an electrical resistance wire wound on the muffle and a refractory cement, especially Alundum cement, covering the resistance wire.

When the furnace is operated at elevated temperatures, such as heat treating temperatures, especially at temperatures of the order of 1400° C. and higher, the refractory materials, particularly the refractory cement, are subject to cracking whereby the winding is exposed and deleteriously affected. The cracking is particularly severe when the furnace temperatures are rapidly elevated and lowered.

For high temperature applications such as described above, the resistance wire employed is advantageously composed of the platinum group metals, for example platinum, and alloys of these metals, in view of the desirable resistance characteristics of such metals at high temperatures. However, in view of the cracking of the muffle and the refractory cement the platinum winding is exposed and the platinum volatilizes, whereby the electrical properties of the winding are no longer maintained constant.

It is an object of the present invention to provide an electrical resistance device for high temperature application. It is another object of the present invention to provide an electrically heated furnace muffle comprising a winding adapted to maintain substantially constant electrical operating characteristics. It is a further object of the present invention to provide a furnace muffle including a resistance winding thereon which is covered by a coat of particular refractory material whereby the winding is effectively protected against volatilization. Other objects and advantages of the invention will become apparent from the description hereinafter following and the drawings forming a part hereof, in which:

FIGURE 1 illustrates a longitudinal sectional view of a furnace muffle with an exposed winding thereon, and

FIGURE 2 illustrates a longitudinal sectional view of a furnace muffle with the winding coated and embedded according to the invention.

In accordance with the invention the resistance wires of the muffle furnace, which are embedded in refractory material, are protected against volatilization and deterioration under high temperatures by means of a particular barrier coating between the metal resistance winding and the refractory material, the barrier coating itself being a particular refractory material, and the winding being composed preferably of a platinum group metal or alloys thereof.

Referring to FIGURE 1, a tubular member 1 composed of a refractory material such as Alundum or zirconium oxide is covered over a major portion of its external surface area with a thin layer 2 of fused aluminum oxide which is deposited on the tubular member 1 while in the molten or fused state and which, on solidification, provides a dense coating integral with the said tubular member. A resistance winding 3 composed of a metal of the platinum group or an alloy composed of metals of

## 2

the platinum group is cleaned and roughened by conventional means and wound over the coating 2. Having provided the winding 3 on the layer 2, the winding and at least a portion of the layer 2, is provided with a further coating 4 of the fused aluminum oxide which effectively combines with the layer 2 of the same material to embed the winding 3 within a thin coat of the integrally combined layers 2 and 4 of fused and solidified aluminum oxide. Subsequently, the coated winding is further coated with a layer 5 of Alundum cement or equivalent refractory cement to complete the furnace muffle. The muffle so constructed effectively protects the volatilization of the winding 3 should any cracking occur in the refractory cement 5. It is of critical significance that the winding 3 is roughened prior to embedding in the combined layers 2 and 4 since the combined layers are substantially thin, of the order of between 0.001" to 0.03", to permit some expansion of the winding 3 without fracture of the embedding layers which are tenaciously mechanically bonded to the roughened windings. Without the embedding or barrier layer composed of the combined layers 2 and 4, the windings would be exposed to the Alundum cement the composition of which is, for example, 90 parts  $\text{Al}_2\text{O}_3$ —5 parts  $\text{SiO}_2$ —5 parts  $\text{CaO}$ , whereby under heated conditions the  $\text{SiO}_2$  reduces in the presence of a platinum group metal forming silicon which reacts with the platinum group metal with deleterious electrical and mechanical effects causing erosion or volatilization of the metal and lowering the melting point thereof.

30 The fused aluminum oxide according to the invention is either aluminum oxide in a substantially pure state or aluminum oxide containing not more than five percent of at least one refractory oxide such as titanium dioxide, calcium oxide, zirconium oxide and the like, with less than one percent  $\text{SiO}_2$ , which amount of  $\text{SiO}_2$  is of critical significance and below the deleterious  $\text{SiO}_2$  content of the Alundum cement, whereby the fused aluminum oxide layer acts as an effective barrier against the  $\text{SiO}_2$  content of the Alundum cement and whereby the effective life of the winding is increased more than five times that of a winding in contact with the Alundum cement.

40 The layers 2 and 4, while shown separately as two layers divided by the dotted line 6, constitute in fact a single integral layer applied in two steps, the last applied fused layer 4 being bonded by fusion with the first applied layer 2.

45 In application, the layers are applied by feeding aluminum oxide powder into a hot flame, where the powder is fused, for example, by an oxygen-acetylene flame and, while in the molten or fused state, is sprayed onto the tube 1 and roughened winding 3 substantially in the manner of producing fused quartz by melting and spraying quartz powder onto a fused quartz base which is well known in the art.

50 While the invention is particularly described and illustrated in connection with a muffle type furnace, it is intended to include herein electrical components such as resistance heated members which constitute a platinum group metal mounted on or contacting  $\text{SiO}_2$  containing material which would normally be deleterious to the metal, and with the barrier layer hereinabove described as a barrier layer between the metal and the support and which is within the scope of the appended claims.

55 What I claim is:

60 1. The method of making a resistance heated member comprising flame spraying an aluminum oxide first coating on a surface of a silica containing refractory support, mounting a metal taken from the group consisting of platinum group metals and alloys thereof on the sprayed surface, and flame spraying a further coating of aluminum oxide on the metal and said first coating thereby embedding the metal in fused aluminum oxide.

2. The method of making a resistance heated member comprising flame spraying molten aluminum oxide to form a first coating on a surface of a silica containing refractory support, winding a wire composed of a metal selected from the group consisting of platinum group metals and alloys thereof over the sprayed surface, and further flame spraying molten aluminum oxide on the wire and said first coating thereby embedding the wire in fused aluminum oxide.

3. The method according to claim 2, wherein the refractory support is a furnace muffle.

4. The method according to claim 2, comprising applying a layer of Alundum cement over the aluminum oxide embedding the wire.

5. The method according to claim 2, wherein the alu-

minum oxide embedding said wire is applied to provide a thickness thereof of from 0.001" to 0.03".

References Cited in the file of this patent

UNITED STATES PATENTS

|           |                |               |
|-----------|----------------|---------------|
| 457,828   | Morford        | Aug. 18, 1891 |
| 1,096,414 | Coolidge       | May 12, 1914  |
| 1,158,972 | Boeck          | Nov. 2, 1915  |
| 1,298,421 | Thomson        | Mar. 25, 1919 |
| 1,802,892 | Hansen         | Apr. 28, 1931 |
| 2,088,949 | Fekete         | Aug. 3, 1937  |
| 2,661,385 | Lincoln et al. | Dec. 1, 1953  |
| 2,961,335 | Shepard        | Nov. 22, 1960 |

FOREIGN PATENTS

|         |               |               |
|---------|---------------|---------------|
| 649,398 | Great Britain | Jan. 24, 1951 |
|---------|---------------|---------------|